

July 15, 1958

J. W. LODGE

2,843,512

METHOD OF RELIEVING BAUSCHINGER EFFECT IN OIL WELL DRILL PIPE

Filed March 24, 1955

20 Sheets-Sheet 1

Fig. I.



TENSILE PROPERTIES OF STEEL SPECIMENS PRESTRAINED VARIOUS AMOUNTS IN COMPRESSION BEFORE TESTING.

Inventor  
JOSEPH W. LODGE

*by Joseph Lemire - Buel  
his attorney*

July 15, 1958

J. W. LODGE

2,843,512

METHOD OF RELIEVING BAUSCHINGER EFFECT IN OIL WELL DRILL PIPE

Filed March 24, 1955

20 Sheets-Sheet 2

Fig. 2.



TENSION AND COMPRESSION YIELD STRENGTH OF STEEL  
PLASTICALLY PRESTRAINED VARIOUS AMOUNTS IN  
COMPRESSION BEFORE TESTING

Inventor

JOSEPH W. LODGE

*by Joseph, Lerner & Bissell  
his attorney*

July 15, 1958

J. W. LODGE

2,843,512

METHOD OF RELIEVING BAUSCHINGER EFFECT IN OIL WELL DRILL PIPE

Filed March 24, 1955

20 Sheets-Sheet 3

Fig. 3.



SHOWS THE EFFECT OF TEMPERATURE ON THE SHAPE OF THE  
TENSILE STRESS-STRAIN CURVE FOR STEEL PRESTRAINED 0.3  
PER CENT IN COMPRESSION

Inventor

JOSEPH W. LODGE

*by Joseph, Leonard & Bule  
his attorney*

July 15, 1958

J. W. LODGE

2,843,512

METHOD OF RELIEVING BAUSCHINGER EFFECT IN OIL WELL DRILL PIPE

Filed March 24, 1955

20 Sheets-Sheet 4

Fig. 4.



SHOWS THE EFFECT OF TEMPERATURE ON THE SHAPE OF THE  
TENSILE STRESS STRAIN-CURVE FOR STEEL PRESTRAINED 0.3  
PER CENT IN COMPRESSION

Inventor

JOSEPH W. LODGE

*by Joseph, Lennard & Selle  
his attorney*

July 15, 1958

J. W. LODGE

2,843,512

METHOD OF RELIEVING BAUSCHINGER EFFECT IN OIL WELL DRILL PIPE

Filed March 24, 1955

20 Sheets-Sheet 5

Fig. 5.



SHOWS THE EFFECT OF TEMPERATURE ON THE SHAPE OF THE  
TENSILE STRESS-STRAIN CURVE FOR STEEL PRESTRAINED 1.5-2.0  
PER CENT IN COMPRESSION

Inventor

JOSEPH W. LODGE

*by Joseph Lemire-Bull  
his attorney*

July 15, 1958

J. W. LODGE

2,843,512

METHOD OF RELIEVING BAUSCHINGER EFFECT IN OIL WELL DRILL PIPE

Filed March 24, 1955

20 Sheets-Sheet 6

Fig. 6.



THE EFFECTS OF HEAT TREATMENTS ON THE TENSILE YIELD  
STRENGTH (0.5 PER CENT TOTAL) FOLLOWING VARIOUS AMOUNTS  
OF PLASTIC PRESTRAIN IN COMPRESSION

Inventor

JOSEPH W. LODGE

*by Joseph, Lennard & Bull  
his attorney*

July 15, 1958

J. W. LODGE

2,843,512

METHOD OF RELIEVING BAUSCHINGER EFFECT IN OIL WELL DRILL PIPE

Filed March 24, 1955

20 Sheets-Sheet 7

Fig. 7.



THE EFFECTS OF VARIOUS TEMPERATURES ON THE TENSILE  
PROPERTIES OF STEEL PRESTRAINED ONE PER CENT OR MORE  
IN COMPRESSION

Inventor

JOSEPH W. LODGE

*by Joseph, Leonard & Bell  
his attorneys*

July 15, 1958

J. W. LODGE

2,843,512

METHOD OF RELIEVING BAUSCHINGER EFFECT IN OIL WELL DRILL PIPE

Filed March 24, 1955

20 Sheets-Sheet 8

Fig. 8.



MECHANICAL PROPERTIES OF TUBING RECEIVING VARIOUS THERMAL AND MECHANICAL TREATMENTS BEFORE TESTING IN TENSION

Inventor

JOSEPH W. LODGE

*by Joseph, Leonard - Buel  
his attorney*

July 15, 1958

J. W. LODGE

2,843,512

METHOD OF RELIEVING BAUSCHINGER EFFECT IN OIL WELL DRILL PIPE

Filed March 24, 1955

20 Sheets-Sheet 9

Fig. 9.



MECHANICAL PROPERTIES OF SAMPLE H1

Inventor

JOSEPH W. LODGE

*by Joseph Leonard Lodge  
his attorney*

July 15, 1958

J. W. LODGE

2,843,512

METHOD OF RELIEVING BAUSCHINGER EFFECT IN OIL WELL DRILL PIPE

Filed March 24, 1955

20 Sheets-Sheet 10

Fig. 10.



MECHANICAL PROPERTIES OF SAMPLE H2

Inventor

JOSEPH W. LODGE

*by Joseph, Leonard & Bule  
his attorney*

July 15, 1958

J. W. LODGE

2,843,512

METHOD OF RELIEVING BAUSCHINGER EFFECT IN OIL WELL DRILL PIPE

Filed March 24, 1955

20 Sheets-Sheet 11

Fig. 11.



MECHANICAL PROPERTIES OF SAMPLE H3

Inventor

JOSEPH W. LODGE

*by Joseph W. Lodge, Esq.  
his attorney*

July 15, 1958

J. W. LODGE

2,843,512

METHOD OF RELIEVING BAUSCHINGER EFFECT IN OIL WELL DRILL PIPE

Filed March 24, 1955

20 Sheets-Sheet 12

Fig. 12.



MECHANICAL PROPERTIES OF SAMPLE H4

Inventor  
JOSEPH W. LODGE

by / Joseph, Lemire & Bell  
his attorney

July 15, 1958

J. W. LODGE

2,843,512

METHOD OF RELIEVING BAUSCHINGER EFFECT IN OIL WELL DRILL PIPE

Filed March 24, 1955

20 Sheets-Sheet 13

Fig. 13.



MECHANICAL PROPERTIES OF SAMPLE H5

Inventor

JOSEPH W. LODGE

by / Joseph, Leonard - Buele  
his attorney

July 15, 1958

J. W. LODGE

2,843,512

METHOD OF RELIEVING BAUSCHINGER EFFECT IN OIL WELL DRILL PIPE

Filed March 24, 1955

20 Sheets-Sheet 14

Fig. 14.



MECHANICAL PROPERTIES OF SAMPLE H6

Inventor

JOSEPH W. LODGE

by /  
Lorraine - Buse  
his attorney

July 15, 1958

J. W. LODGE

2,843,512

METHOD OF RELIEVING BAUSCHINGER EFFECT IN OIL WELL DRILL PIPE

Filed March 24, 1955

20 Sheets-Sheet 15

Fig. 15.



TENSILE PROPERTIES OF STEEL TUBING WHICH  
HAD BEEN PREVIOUSLY SUBJECT TO FATIGUE -  
TYPE LOADING

Inventor

JOSEPH W. LODGE

by / Joseph, Lemire, Bucci  
his attorney

July 15, 1958

J. W. LODGE

2,843,512

METHOD OF RELIEVING BAUSCHINGER EFFECT IN OIL WELL DRILL PIPE

Filed March 24, 1955

20 Sheets-Sheet 16

Fig. 16.



COMPRESSION PROPERTIES OF STEEL TUBING  
WHICH HAD BEEN PREVIOUSLY SUBJECT TO  
FATIGUE-TYPE LOADING

Inventor

JOSEPH W. LODGE

*by Joseph W. Lodge, Lorraine E. Bell  
his attorney*

July 15, 1958

J. W. LODGE

2,843,512

METHOD OF RELIEVING BAUSCHINGER EFFECT IN OIL WELL DRILL PIPE

Filed March 24, 1955

20 Sheets-Sheet 17

Fig. 17.



MECHANICAL PROPERTIES OF STEEL IN NORMALIZED CONDITION  
TESTED ALTERNATELY IN TENSION AND COMPRESSION THROUGH  
A RANGE OF STRAIN OF APPROXIMATELY 0.5 PER CENT

Inventor  
JOSEPH W. LODGE

*by Joseph, Leonard & Buell  
his attorney*

July 15, 1958

J. W. LODGE

2,843,512

METHOD OF RELIEVING BAUSCHINGER EFFECT IN OIL WELL DRILL PIPE

Filed March 24, 1955

20 Sheets-Sheet 18

Fig. 18.



MECHANICAL PROPERTIES OF STEEL IN NORMALIZED CONDITION  
TESTED ALTERNATELY IN TENSION AND COMPRESSION THROUGH  
A RANGE OF STRAIN OF APPROXIMATELY 0.5 PER CENT

Inventor

JOSEPH W. LODGE

*by / Joseph, Leonard - Buse  
his attorney*

July 15, 1958

J. W. LODGE

2,843,512

METHOD OF RELIEVING BAUSCHINGER EFFECT IN OIL WELL DRILL PIPE

Filed March 24, 1955

20 Sheets-Sheet 19

Fig. 19



MECHANICAL PROPERTIES OF STEEL IN NORMALIZED CONDITION  
TESTED ALTERNATELY IN TENSION AND COMPRESSION THROUGH  
A RANGE OF STRAIN OF APPROXIMATELY 1.0 PER CENT

Inventor

JOSEPH W. LODGE

*by Joseph, Lorraine & Buell  
his attorney*

July 15, 1958

J. W. LODGE

2,843,512

METHOD OF RELIEVING BAUSCHINGER EFFECT IN OIL WELL DRILL PIPE

Filed March 24, 1955

20 Sheets-Sheet 20

Fig. 20.



MECHANICAL PROPERTIES OF STEEL IN NORMALIZED CONDITION  
TESTED ALTERNATELY IN COMPRESSION AND TENSION THROUGH  
A RANGE OF STRAIN OF APPROXIMATELY 1.0 PER CENT

Inventor

JOSEPH W. LODGE

*by / Joseph, Leonard - Knell  
his attorney*

1

2,843,512

**METHOD OF RELIEVING BAUSCHINGER EFFECT  
IN OIL WELL DRILL PIPE**

Joseph W. Lodge, Sharon Township, Franklin County, Ohio, assignor, by mesne assignments, to The Youngstown Sheet and Tube Company, Youngstown, Ohio, a corporation of Ohio

Application March 24, 1955, Serial No. 496,392

3 Claims. (Cl. 148—4)

This invention relates to a method of relieving the Bauschinger effect in metal, particularly a method which is well adapted for field use and does not require high temperature heat treatment such as normalizing.

The Bauschinger effect, as known to metallurgists, is the reduction in one direction of properties of metal subjected to cold plastic deformation in another direction. For example, the elastic limit and yield strength in tension of a specimen of metal which is subjected to cold plastic deformation by compression generally along the axis of testing are reduced relatively to the original elastic limit and yield strength of the metal in tension. The reduction in elastic limit and yield strength is due to microstresses set up within the atomic lattice of the metal. Such stresses are to be distinguished from macrostresses which are customarily relieved by normalizing.

I have devised a method of treating metal which due to cold plastic deformation of the metal contains within the atomic lattice microstresses which decrease the elastic limit and yield strength of the metal in the direction opposite the direction of the cold plastic deformation relatively to the elastic limit and yield strength in that direction of the metal prior to the cold plastic deformation, comprising at least substantially restoring the original elastic limit and yield strength of the metal by applying thereto energy relieving the microstresses within the atomic lattice. The energy may be applied in the form of heat energy or in the form of mechanical energy. When the metal being treated is steel and the energy applied is in the form of heat energy I preferably heat treat the steel at a temperature in the range 400—1250° F. whereby I relieve the microstresses within the atomic lattice. I prefer to heat treat steel at about 850° F. for about an hour although good results are obtained at lower and higher temperatures. In general the time of heat treatment varies inversely with the temperature although the time-temperature relationship is not necessarily a straight line relationship.

My invention has various practical applications, one of which is the relief of the Bauschinger effect in drill pipe in the field without requiring the use of a closely controlled normalizing furnace. I find that I can relieve the Bauschinger effect by a heat treatment at a substantially lower temperature and for a shorter time than the heat treatment required for normalizing; also that the time, temperature and cooling rate are less critical than in normalizing. I find that I can even improve on

2

the original properties of metal having the Bauschinger effect. In some cases the metal after my treatment may not have quite as good properties as it had originally but its properties may be improved sufficiently to meet specifications through a simple treatment which can be performed in the field with comparatively inexpensive apparatus. This is in contra-distinction to prior practice which has been to ship the pipe, often hundreds of miles, to a heat treating plant for normalizing.

10 Other details, objects and advantages of the invention will become apparent as the following description of certain present preferred methods of practicing the same proceeds.

15 The drawings—Figures 1 to 20, inclusive—are all charts or graphs showing the effect of various treatments upon described specimens, each chart being fully explained by its title and the legends appearing therein.

A series of samples of grade E seamless drill pipe were strained by compression loads producing permanent sets ranging from 1% to 2.5%. Tensile tests made on conventional test bars prepared from the pipe samples prestrained a minimum of 1% show a 30% loss in yield strength as measured at 5% total elongation. The first 5% of prestrain is the most effective in lowering the yield strength and establishes 75% of the maximum loss in strength over the range of prestrain values investigated. The compression tests, in which the steel was strained in the same direction as the prestraining, show yield strength values increasing in proportion to the amount of prestrain to about 1% with only a very slight gain in strength from about 1% to about 2.5% prestrain. This directional gain in strength is the one normally thought of as the effect of cold working a metal.

35 The magnitude of the Bauschinger effect depends upon the condition of the metal before prestraining. Normalized steel pipe heated to 1250° F. for one hour before prestraining 1.5% at room temperature showed a loss in yield strength in tension of greater than 50% as compared to a 30% loss for the normalized sample prestrained the same amount.

40 Prestraining in a direction opposite to the direction of subsequent testing has a very pronounced effect upon the shape of the stress-strain curve. The curve shows that the metal loses its elastic characteristics at a relatively low stress level. Above the elastic limit the curve has a large radius of curvature. This is a type of curve which results from the averaging effect of unequal distribution of the internal stresses superimposed on the applied stress. Because the effect is greater than normally encountered with familiar residual stress conditions it suggests that prestraining produces directional internal stresses within the atomic lattice or along grain boundaries.

45 I have found that the elastic property can be restored to the metal by a one hour heat treatment at a temperature which may be as low as 400° F. Higher temperatures appear to have a combined stress-relieving and strain aging effect. Optimum properties are obtained by heat treatment for about one hour at a temperature

of the order of 850° F. However, the effects of the heat treatment are dependent upon both time and temperature.

Three samples of drill pipe which had seen field service showed a large Bauschinger effect in compression tests. The elastic properties were restored and the yield strength of the samples was raised well above the specification minimum by my method.

Tests conducted on a pipe containing a moderate amount of residual internal stress show that the elastic properties are restored in fatigue-type loading if the applied stresses are sufficiently high. The pipe was loaded as a cantilever beam and rotated 26,000 revolutions. The elastic properties were restored in samples cut from a location in the pipe stressed to 31,500 pounds per square inch (hereinafter abbreviated "p. s. i.") in the outer fibers but not in samples which were stressed to only 16,500 p. s. i. in the outer fibers.

Two lengths of 5-inch outside diameter 19.50-pound grade E seamless steel drill pipe were tested. Such lengths of drill pipe did not receive special processing and may be regarded as representative of regular production pipe which has been normalized and rotary straightened. The analyses and properties of the metal are set forth in Table 1.

sample from each load was tested to determine the mechanical properties after normalizing. The purpose of the normalizing treatment was to avoid the possibility that variable amounts of residual strain introduced by the rotary straightener might remain. The two ends of each sample were accurately ground to produce parallel surfaces normal to the longitudinal axis of the pipe.

A series of the pipe samples were strained in compression various amounts to produce permanent sets ranging from .1% to 2.5%. A hydraulic press having a rated capacity of 700 tons was used to compress the pipe samples. A load of approximately 300 tons was required to exceed the elastic limit.

During the compression loading the change in length of the samples was measured with a dial gauge placed between the face plates on the press, and the strain was measured also with a Baldwin SR-4 type electric strain gauge placed at the center of the length of the sample. Because of friction between the ends of the samples and the face plates of the press the average strain over the entire length of a specimen was less than the strain at the center of its length. The SR-4 gauge was used to control the amount of permanent set in the sample because it was disposed at the location of the gauge length of conventional tensile and compression test bars subsequently cut from the pipe samples. Measurements of the diameter of the pipe samples also showed a greater increase in diameter at the center than near the ends.

After prestraining in compression conventional tensile and compression test bars were machined from longitudinal strips sawed from the pipe samples. The tensile bars were one inch wide at the grip ends with a reduced section  $\frac{3}{4}$  inch wide and  $2\frac{1}{2}$  inches long. Because of the relatively small radius of curvature of the pipe the thickness of the tensile specimens was limited to .2 inch. The tensile bars were tested in a standard Baldwin testing machine using "Templin" self-aligning grips. The strain was measured with a pair of Baldwin SR-4 type A3 electric strain gauges cemented to the opposite surfaces at the center of the gauge length. The compression bars were  $1\frac{1}{2}$  inches in length with a rectangular cross section measuring approximately .3" x .45". A subpress was used with the Baldwin testing machine to establish and maintain alignment in testing the compression bars. The strain was measured with a pair of type A7 gauges cemented to the .45 inch faces of the bars.

The results of the compression and tensile tests on specimens with various amounts of plastic prestrain are given in Table 2. The effect that various amounts of plastic strain in compression have on the properties of the steel as subsequently determined in tensile tests is shown graphically in Figure 1. The stress-strain curve for the normalized material, which is representative of all of the samples before prestraining, is straight to a stress of approximately 80,000 p. s. i., indicating elastic behavior to that stress level. The fairly sharp turn and moderate slope of the curve above 80,000 p. s. i. indicate that substantially all of the fibers throughout the cross section yielded at essentially the same stress level and that the metal work hardened to some extent in the plastic

TABLE 1

## Chemical composition and mechanical properties

[Composition, percent]

| C                                          | Mn     | P                                      | S       | Si                                 | Mo   |
|--------------------------------------------|--------|----------------------------------------|---------|------------------------------------|------|
| Ladle Analysis                             |        |                                        |         |                                    |      |
| 0.38                                       | 1.58   | 0.028                                  | 0.022   | 0.23                               | 0.18 |
| 0.38                                       | 1.58   | 0.030                                  | 0.021   | --                                 | --   |
| Check Analysis                             |        |                                        |         |                                    |      |
| 0.40                                       | 1.60   | 0.031                                  | 0.019   | 0.20                               | 0.18 |
| 0.39                                       | 1.60   | 0.026                                  | 0.019   | 0.21                               | 0.18 |
| Yield Strength,<br>0.5% Total,<br>p. s. i. |        | Ultimate Tensile Strength,<br>p. s. i. |         | Elongation in 2 Inches,<br>percent |      |
| 60,030                                     | 83,330 | 127,450                                | 122,850 | 26.0                               | 26.0 |

The drill pipe described above was cut into lengths approximately ten inches long. That length was selected as a convenient length for the tensile test bars which were to be cut from the pipes. That length also provides a favorable diameter-length ratio to avoid buckling under axial compression. All of the 10-inch long samples were normalized by heating them to 1600° F. and air cooling. The normalizing was done in two furnace loads. One

range. On the other hand the curves representing the prestrained metal leave the elastic range at a very low stress level and form long sweeping curves which are progressively lower with increasing amount of prestrain.

a directional weakness that will make the pipe easier to bend or kink in service if the stress field is reversed. A straightening operation will also work the metal plastically and establish other directional weaknesses. Al-

TABLE 2  
*Mechanical properties of steel specimens prestrained in compression before testing*

| Specimen Number | Plastic Pre-strained percent | Compression Yield Strength |                      |                     | Tensile Yield Strength |                      |                     | Ultimate Tensile Strength p. s. i. | Elongation percent |
|-----------------|------------------------------|----------------------------|----------------------|---------------------|------------------------|----------------------|---------------------|------------------------------------|--------------------|
|                 |                              | 0.02% Offset p. s. i.      | 0.2% Offset p. s. i. | 0.5% Total p. s. i. | 0.02% Offset p. s. i.  | 0.2% Offset p. s. i. | 0.5% Total p. s. i. |                                    |                    |
| G11.....        | 0                            | 67,000                     | 105,000              | 103,000             | 69,000                 | 86,000               | 87,000              | 123,500                            | 21                 |
|                 | 0                            | -----                      | -----                | -----               | 58,000                 | 84,000               | 84,500              | 122,500                            | 17                 |
| G17.....        | 0                            | -----                      | -----                | -----               | 76,000                 | 88,000               | 88,000              | 118,500                            | 20                 |
|                 | 0                            | -----                      | -----                | -----               | 82,000                 | 88,000               | 88,500              | 120,000                            | 19                 |
| G2.....         | 0.1                          | 94,500                     | 98,000               | 98,500              | 38,500                 | 80,500               | 82,000              | 120,500                            | 18                 |
|                 | 0.1                          | -----                      | -----                | -----               | 44,000                 | 82,000               | 83,500              | 123,000                            | 19                 |
| G8.....         | 0.2                          | 98,000                     | 103,500              | 104,000             | 37,500                 | 79,000               | 81,000              | 122,500                            | 18                 |
|                 | 0.2                          | -----                      | -----                | -----               | 39,500                 | 76,000               | 79,500              | 122,000                            | 17                 |
| G3.....         | 0.3                          | 100,500                    | 105,000              | 105,000             | 33,000                 | 70,000               | 75,000              | 123,000                            | 17                 |
|                 | 0.3                          | -----                      | -----                | -----               | 31,000                 | 68,500               | 74,000              | 121,000                            | 18                 |
| G10.....        | 0.4                          | 99,000                     | 104,500              | 103,500             | 32,000                 | 67,000               | 72,000              | 119,000                            | 19                 |
|                 | 0.4                          | -----                      | -----                | -----               | 23,000                 | 66,500               | 72,000              | 121,500                            | 21                 |
| G6.....         | 0.5                          | 99,000                     | 106,500              | 106,000             | 26,000                 | 60,000               | 67,000              | 120,000                            | 20                 |
|                 | 0.5                          | -----                      | -----                | -----               | 30,000                 | 61,500               | 68,000              | 120,000                            | 18                 |
| G4.....         | 0.75                         | 105,000                    | 112,500              | 112,000             | 26,000                 | 59,000               | 66,000              | 122,500                            | 22                 |
|                 | 0.75                         | -----                      | -----                | -----               | 26,000                 | 58,000               | 65,000              | 121,500                            | 19                 |
| G5.....         | 1.0                          | 113,000                    | 121,500              | 121,000             | 26,000                 | 55,000               | 62,000              | 118,500                            | 22                 |
|                 | 1.0                          | -----                      | -----                | -----               | 26,000                 | 55,000               | 62,500              | 119,000                            | 21                 |
| G7.....         | 1.5                          | 108,000                    | 121,500              | 120,000             | 26,500                 | 55,000               | 62,000              | 119,000                            | 21                 |
|                 | 1.5                          | -----                      | -----                | -----               | 27,000                 | 55,000               | 62,000              | 119,500                            | 20                 |
| G1.....         | 2.0                          | 118,000                    | 123,000              | 122,000             | 26,000                 | 55,000               | 62,000              | 120,000                            | 22                 |
|                 | 2.0                          | -----                      | -----                | -----               | 30,000                 | 56,000               | 62,000              | 120,000                            | 20                 |
| G9.....         | 2.5                          | 102,000                    | 125,000              | 122,000             | 25,500                 | 54,000               | 61,000              | 117,500                            | 23                 |
|                 | 2.5                          | -----                      | -----                | -----               | 30,000                 | 55,500               | 62,000              | 118,000                            | 18                 |

<sup>1</sup> Failed outside of gauge marks.

NOTE.—All pipe samples normalized before prestraining.

In this respect the Bauschinger effect is similar to the effect of residual stresses of a macroscopic nature such as are introduced by unequal rates of expansion or contraction in heating or cooling a part. However, the effects shown in Figure 1 seem much too large to be accounted for by the residual stresses ordinarily encountered, and it is believed that at least part of the effect is the result of directional residual stresses of a microscopic nature introduced by prestraining in a direction opposite to that used in testing.

The low sweep of the curve results in lower yield strength, as arbitrarily measured at .5% elongation and even lower values if measured by the .2% offset method. However, the elastic limit is depressed to a small fraction of its initial value. This is particularly important from the standpoint of bending under service conditions. The values for ultimate tensile strength and elongation as shown in Table 2 are not significantly different for the bars having various amounts of prestrain. This can be interpreted as evidence that the Bauschinger effect is a complex but directional residual stress condition.

Figure 2 shows the effect of various amounts of prestrain on both compression and tensile yield strengths. Note that the maximum reduction of yield strength is established at about 1% and remains at that level up to and including about 2.5% prestrain. Furthermore approximately 75% of the effect in tension is established with only .5% prestrain. There is a general symmetry between the curves representing the compression and tensile yield strengths in Figure 2. The compression yield strength is raised by increasing amounts of prestrain, also reaching a maximum rate at approximately 1%. This is the strengthening effect normally associated with cold work.

The results show that plastic cold work will establish

though it is known to those skilled in the art that a normalizing heat treatment will reestablish the original properties such has not been the case with respect to the lower temperature more practical treatment which I employ.

Additional compression and tensile test bars were prepared from the same series of prestrained pipe samples whose test results are described above. The additional test bars were heat treated at various temperature levels ranging from 250° F. to 1250° F., inclusive. The results of compression and tensile tests on those bars following the various heat treatments are set forth in Tables 3 to 6, inclusive.

The effect of temperature on the shape of the tensile stress-strain curve for the normalized pipe prestrained .3% in compression before the heat treatment is shown graphically in Figures 3 and 4, and for prestrain of 1.5% to 2% in Figure 5. At both levels of strain the effects of the heat treatment are similar. The stress-strain curves for the bars treated at 250° F. are similar in shape to those for corresponding prestrain values but with all stress values at given strains somewhat higher. Apparently the treatment produces a mild strain aging effect. However, the 400° F. treatment restored the elastic characteristics to the steel up to a stress level a little over 70,000 p. s. i. Higher temperatures restore the elastic characteristics to higher stress levels and raise the yield strength, reaching optimum values at approximately 850° F. Apparently temperatures in that range have the combined effect of strain aging and release of both residual macrostresses and microstresses. Although temperatures in the range 850–1250° F. restore the elastic characteristics the yield strength is lowered progressively with increasing temperatures. A holding time of one hour in that temperature range appears to produce an overaged condition.

TABLE 3  
*Mechanical properties of steel specimens prestrained in compression and heat treated before testing in tension*

| Specimen Number | Plastic Pre-strained, percent | Temp., F. | Compression Yield Strength |                       |                      | Tensile Yield Strength |                       |                      | Ultimate Tensile Strength, p. s. i. | Elongation, percent |
|-----------------|-------------------------------|-----------|----------------------------|-----------------------|----------------------|------------------------|-----------------------|----------------------|-------------------------------------|---------------------|
|                 |                               |           | 0.02% Offset, p. s. i.     | 0.2% Offset, p. s. i. | 0.5% Total, p. s. i. | 0.02% Offset, p. s. i. | 0.2% Offset, p. s. i. | 0.5% Total, p. s. i. |                                     |                     |
| U11             | 0                             | 250       | 75,000                     | 105,000               | 103,500              | 71,000                 | 92,000                | 92,000               | 123,000                             | 17                  |
|                 | 0                             | 250       | 70,000                     | 88,500                | 88,500               | 70,000                 | 88,500                | 88,500               | 123,500                             | 19                  |
| U17             | 0                             | 250       | —                          | —                     | —                    | —                      | —                     | —                    | —                                   | —                   |
|                 | 0                             | 250       | —                          | —                     | —                    | —                      | —                     | —                    | —                                   | —                   |
| U2              | 0.1                           | 250       | 96,000                     | 97,000                | 98,000               | 47,500                 | 82,000                | 83,000               | 121,500                             | 18                  |
|                 | 0.1                           | 250       | 66,000                     | 90,000                | 88,500               | 42,000                 | 72,000                | 75,500               | 123,000                             | 20                  |
| U8              | 0.2                           | 250       | 94,000                     | 98,500                | 98,000               | 48,000                 | 84,500                | 85,000               | 121,000                             | 18                  |
|                 | 0.2                           | 250       | 49,000                     | 84,000                | 85,000               | 49,000                 | 84,000                | 85,000               | 123,000                             | 17                  |
| U3              | 0.3                           | 250       | 82,500                     | 104,000               | 104,000              | 42,000                 | 73,500                | 76,500               | 122,000                             | 19                  |
|                 | 0.3                           | 250       | 45,500                     | 76,000                | 79,000               | 45,500                 | 76,000                | 79,000               | 121,500                             | 17                  |
| U10             | 0.4                           | 250       | 99,000                     | 104,000               | 104,000              | 40,000                 | 72,000                | 75,500               | 121,500                             | 21                  |
|                 | 0.4                           | 250       | 42,000                     | 72,500                | 76,000               | 42,000                 | 72,500                | 76,000               | 120,500                             | 19                  |
| U6              | 0.5                           | 250       | 97,000                     | 105,000               | 104,500              | 36,000                 | 66,000                | 71,000               | 121,000                             | 18                  |
|                 | 0.5                           | 250       | 40,000                     | 66,000                | 70,500               | 40,000                 | 66,000                | 70,500               | 121,500                             | 17                  |
| U4              | 0.75                          | 250       | 90,000                     | 112,000               | 111,500              | 35,000                 | 64,000                | 69,000               | 121,500                             | 19                  |
|                 | 0.75                          | 250       | 41,000                     | 65,000                | 70,000               | 41,000                 | 65,000                | 70,000               | 123,000                             | 20                  |
| U5              | 1.0                           | 250       | 85,000                     | 118,000               | 118,000              | 34,500                 | 61,000                | 66,500               | 119,000                             | 21                  |
|                 | 1.0                           | 250       | 38,000                     | 62,000                | 67,000               | 38,000                 | 62,000                | 67,000               | 120,000                             | 20                  |
| U7              | 1.5                           | 250       | 100,000                    | 121,500               | 121,000              | 34,500                 | 60,500                | 66,000               | 118,500                             | 19                  |
|                 | 1.5                           | 250       | 37,000                     | 60,000                | 65,500               | 37,000                 | 60,000                | 65,500               | 118,500                             | 21                  |
| U1              | 2.0                           | 250       | 115,000                    | 125,000               | 124,500              | 35,000                 | 60,000                | 65,000               | 117,500                             | 21                  |
|                 | 2.0                           | 250       | 30,000                     | 60,000                | 65,500               | 30,000                 | 60,000                | 65,500               | 118,500                             | 19                  |
| U9              | 2.5                           | 250       | 96,000                     | 129,500               | 129,000              | 33,000                 | 60,500                | 65,500               | 118,000                             | 21                  |
|                 | 2.5                           | 250       | 36,000                     | 61,000                | 66,000               | 36,000                 | 61,000                | 66,000               | 119,000                             | 20                  |

NOTE.—All specimens held one hour at temperature.

TABLE 4  
*Tensile properties of steel specimens prestrained in compression and heat treated before testing in tension*

| Specimen Number | Plastic Pre-strained, percent | Temp., F. | Tensile Yield Strength |                       |                      | Ultimate Tensile Strength, p. s. i. | Elongation, percent |
|-----------------|-------------------------------|-----------|------------------------|-----------------------|----------------------|-------------------------------------|---------------------|
|                 |                               |           | 0.02% Offset, p. s. i. | 0.2% Offset, p. s. i. | 0.5% Total, p. s. i. |                                     |                     |
| J11             | 0                             | 400       | 96,000                 | 104,000               | 104,000              | 128,500                             | 16.0                |
| J2              | 0.1                           | 400       | 76,000                 | 91,000                | 91,000               | 124,500                             | 17.0                |
| J3              | 0.3                           | 400       | 68,000                 | 86,000                | 86,000               | 125,000                             | 20.0                |
| J6              | 0.5                           | 400       | 74,000                 | 82,000                | 83,000               | 123,250                             | 17.0                |
| J5              | 1.0                           | 400       | 77,500                 | 82,500                | 83,000               | 123,500                             | 17.0                |
| J1              | 2.0                           | 400       | 77,500                 | 83,000                | 83,000               | 125,000                             | 17.0                |
| X11             | 0                             | 650       | 105,000                | 107,500               | 107,500              | 129,500                             | 17.0                |
| X8              | 0.2                           | 650       | 80,000                 | 90,000                | 90,000               | 123,000                             | 18.0                |
| X10             | 0.4                           | 650       | 86,500                 | 87,000                | 87,000               | 125,000                             | 19.0                |
| X7              | 1.5                           | 650       | 87,500                 | 89,000                | 89,000               | 123,500                             | 17.0                |
| X9              | 2.5                           | 650       | 79,500                 | 87,500                | 87,500               | 124,000                             | 18.0                |
| P8              | 0.2                           | 850       | 92,000                 | 94,000                | 94,000               | 122,500                             | 19.0                |
| P10             | 0.4                           | 850       | 91,500                 | 93,000                | 93,000               | 122,500                             | 18.0                |
| P4              | 0.75                          | 850       | 83,000                 | 90,500                | 90,000               | 121,000                             | 20.0                |
| P7              | 1.5                           | 850       | 93,000                 | 94,500                | 94,500               | 123,000                             | 19.0                |
| P9              | 2.5                           | 850       | 87,000                 | 95,000                | 95,000               | 121,500                             | 19.0                |
| M2              | 0.1                           | 1,050     | 84,000                 | 88,500                | 88,500               | 114,000                             | 23.0                |
| M3              | 0.3                           | 1,050     | 87,000                 | 87,000                | 87,000               | 113,000                             | 22.0                |
| M6              | 0.5                           | 1,050     | 86,500                 | 86,500                | 86,500               | 112,500                             | 23.0                |
| M5              | 1.0                           | 1,050     | 88,000                 | 88,000                | 88,000               | 112,750                             | 23.0                |
| M1              | 2.0                           | 1,050     | 88,000                 | 88,000                | 88,000               | 112,500                             | 21.0                |

NOTE.—All specimens held one hour at temperature.

TABLE 5  
*Tensile properties of steel specimens prestrained in compression and heat treated before testing in tension*

| Specimen Number | Plastic Pre-strained, percent | Temp., F. | Tensile Yield Strength |                       |                      | Ultimate Tensile Strength, p. s. i. | Elongation, percent |
|-----------------|-------------------------------|-----------|------------------------|-----------------------|----------------------|-------------------------------------|---------------------|
|                 |                               |           | 0.02% Offset, p. s. i. | 0.2% Offset, p. s. i. | 0.5% Total, p. s. i. |                                     |                     |
| G12             | 0.3                           | 30,000    | 73,000                 | 74,000                | 120,500              | 21.0                                |                     |
| U12             | 0.3                           | 52,000    | 78,500                 | 80,500                | 119,000              | 18.0                                |                     |
| J12             | 0.3                           | 400       | 78,000                 | 81,500                | 82,000               | 119,500                             | 19.0                |
| B12             | 0.3                           | 700       | —                      | —                     | —                    | —                                   | —                   |
| B12             | 0.3                           | 750       | 89,000                 | 89,500                | 89,500               | 120,000                             | 21.0                |
| P12             | 0.3                           | 850       | 91,000                 | 91,000                | 91,000               | 118,000                             | 21.0                |
| D12             | 0.3                           | 900       | 89,000                 | 89,000                | 89,000               | 116,000                             | 22.0                |
| E12             | 0.3                           | 950       | 87,000                 | 87,000                | 87,000               | 112,500                             | 21.0                |
| G13             | 1.5                           | 23,000    | 57,000                 | 61,000                | 116,000              | 20.0                                |                     |
| U13             | 1.5                           | 250       | 43,000                 | 70,000                | 72,000               | 118,000                             | 20.0                |
| J13             | 1.5                           | 400       | 72,000                 | 80,000                | 81,000               | 121,000                             | 19.0                |
| A14             | 1.5                           | 700       | 88,000                 | 89,000                | 89,000               | 121,500                             | 19.0                |
| B13             | 1.5                           | 750       | 89,500                 | 90,000                | 90,000               | 119,000                             | 20.0                |
| C14             | 1.5                           | 800       | 92,000                 | 93,000                | 93,000               | 118,500                             | 18.0                |
| P13             | 1.5                           | 850       | 90,500                 | 90,500                | 90,500               | 115,500                             | 20.0                |
| D13             | 1.5                           | 900       | 89,000                 | 89,000                | 89,000               | 114,500                             | 22.0                |
| E13             | 1.5                           | 950       | 88,600                 | 88,500                | 88,500               | 113,000                             | 21.0                |

<sup>1</sup> At temperature 16 hours, all other specimens held one hour at temperature.

TABLE 6

*Mechanical properties of steel specimens prestrained in compression and heat treated before testing in tension*

| Specimen Number | Plastic Pre-strained, percent | Temp., F. | Compression Yield Strength |                       |                      | Tensile Yield Strength |                       |                      | Ultimate Tensile Strength, p. s. i. | Elongation, percent |
|-----------------|-------------------------------|-----------|----------------------------|-----------------------|----------------------|------------------------|-----------------------|----------------------|-------------------------------------|---------------------|
|                 |                               |           | 0.02% Offset, p. s. i.     | 0.2% Offset, p. s. i. | 0.5% Total, p. s. i. | 0.02% Offset, p. s. i. | 0.2% Offset, p. s. i. | 0.5% Total, p. s. i. |                                     |                     |
| V11             | 0                             | 1,250     | 82,500                     | 82,500                | 82,500               | 76,000                 | 77,000                | 77,000               | 102,000                             | 25                  |
|                 | 0                             | 1,250     |                            |                       |                      | 77,500                 | 77,500                | 77,500               | 103,000                             | 26                  |
| V17             |                               | 1,250     |                            |                       |                      |                        |                       |                      |                                     |                     |
|                 |                               | 1,250     |                            |                       |                      |                        |                       |                      |                                     |                     |
| V2              | 0.1                           | 1,250     | 82,500                     | 82,500                | 82,500               | 76,000                 | 76,000                | 76,000               | 100,500                             | 25                  |
|                 | 0.1                           | 1,250     |                            |                       |                      | 75,000                 | 76,000                | 76,000               | 101,500                             | 27                  |
| V8              | 0.2                           | 1,250     | 85,500                     | 86,000                | 86,000               | 76,000                 | 76,000                | 76,000               | 101,000                             | 24                  |
|                 | 0.2                           | 1,250     |                            |                       |                      | 75,000                 | 75,500                | 75,500               | 100,000                             | 28                  |
| V3              | 0.3                           | 1,250     | 84,000                     | 84,000                | 84,000               | 76,500                 | 77,000                | 77,000               | 102,000                             | 26                  |
|                 | 0.3                           | 1,250     |                            |                       |                      | 76,000                 | 76,500                | 76,500               | 101,000                             | 27                  |
| V10             | 0.4                           | 1,250     | 85,000                     | 85,000                | 85,000               | 75,000                 | 76,000                | 76,000               | 101,000                             | 27                  |
|                 | 0.4                           | 1,250     |                            |                       |                      | 77,500                 | 77,500                | 77,500               | 103,000                             | 27                  |
| V6              | 0.5                           | 1,250     | 83,000                     | 83,000                | 83,000               | 76,000                 | 76,000                | 76,000               | 101,000                             | 26                  |
|                 | 0.5                           | 1,250     |                            |                       |                      | 76,000                 | 74,500                | 75,000               | 101,000                             | 26                  |
| V4              | 0.75                          | 1,250     | 86,500                     | 86,500                | 86,500               | 77,000                 | 77,000                | 77,000               | 102,000                             | 27                  |
|                 | 0.75                          | 1,250     |                            |                       |                      | 77,000                 | 77,500                | 77,500               | 101,000                             | 27                  |
| V5              | 1.0                           | 1,250     | 82,500                     | 82,000                | 82,500               | 79,000                 | 79,000                | 79,000               | 104,000                             | 25                  |
|                 | 1.0                           | 1,250     |                            |                       |                      | 76,000                 | 76,500                | 76,500               | 101,500                             | 26                  |
| V7              | 1.5                           | 1,250     | 83,000                     | 83,000                | 83,000               | 76,000                 | 76,000                | 76,000               | 100,000                             | 25                  |
|                 | 1.5                           | 1,250     |                            |                       |                      | 76,000                 | 76,000                | 76,000               | 100,000                             | 27                  |
| V1              | 2.0                           | 1,250     | 82,000                     | 82,000                | 82,000               | 78,500                 | 78,500                | 78,500               | 101,000                             | 25                  |
|                 | 2.0                           | 1,250     |                            |                       |                      | 78,500                 | 79,000                | 79,000               | 102,000                             | 27                  |
| V9              | 2.5                           | 1,250     | 87,000                     | 87,000                | 87,000               | 78,000                 | 78,000                | 78,000               | 101,000                             | 26                  |
|                 | 2.5                           | 1,250     |                            |                       |                      | 77,000                 | 76,500                | 76,500               | 99,500                              | 25                  |

NOTE.—All specimens held one hour at temperature.

A summary in graphical form of the effect on tensile yield strength of various heat treating temperatures and various amounts of plastic prestrain in compression before heating is shown in Figure 6. The effect of various temperatures on the tensile properties of the steel prestrained 1% or more in compression before testing is shown in Figure 7. Although the optimum properties are obtained at a temperature near 850° F. all of the heat treatments in the temperature range 400–1250° F. restored the properties to values exceeding the API minimum yield strength of 75,000 p. s. i. for the grade of pipe in question.

Although it has been demonstrated above that a temperature of 850° F. produces optimum properties with a one hour treatment the effect is also dependent upon time. The curve D of Figure 8 evidences that rapid heating to 1050° F. produces equivalent properties and overaging occurs with longer heating times (curves E and F). Curve A indicates a mild residual stress condition in the material as received from the mill and curve B the beneficial effect of a normalizing treatment. Curve G shows that the magnitude of the Bauschinger effect for a given amount of prestrain is dependent upon the condition or thermal history of the metal before prestraining. The yield strength at .5% total strain was lowered an additional 10,000 p. s. i. by heating the pipe at 1250° F. for one hour between the normalizing and prestraining treatments.

Samples from six lengths of crooked pipe which had been used in drilling operations were also tested. Such pipe may have been bent and straightened several times during its field service life. The samples were selected as being representative of the condition of drill pipe in which the yield strength had been found to be lower than the specification minimum values. The six samples were identified by the indicia H1 to H6, inclusive. Drill-

ings from the six samples were analyzed with the results shown in Table 7.

TABLE 7  
35 Results of chemical analysis of used drill pipe samples

| Sample Number | Composition, percent |      |       |       |      |      |
|---------------|----------------------|------|-------|-------|------|------|
|               | C                    | Mn   | P     | S     | Si   | Mo   |
| H1            | 0.39                 | 1.42 | —     | 0.021 | 0.23 | 0.18 |
| H2            | 0.43                 | 1.50 | 0.021 | 0.021 | 0.20 | 0.17 |
| H3            | 0.41                 | 1.42 | 0.018 | 0.021 | 0.21 | 0.18 |
| H4            | 0.40                 | 1.48 | 0.021 | 0.021 | 0.19 | 0.17 |
| H5            | 0.38                 | 1.42 | —     | —     | 0.19 | 0.16 |
| H6            | 0.41                 | 1.50 | 0.020 | —     | 0.19 | 0.18 |

A tensile test bar and duplicate compression test bars were machined from each of the six samples to the same size and shape as described above for similar test bars. The above described testing procedure was used. The test results are given in Table 8. A similar series of test bars was prepared from samples of the pipe that been heated to 850° F. and held at temperature for one hour. This is the most effective heat treatment to restore the elastic properties and obtain the maximum yield strength. The results of tests on these bars are also shown in Table 8. The stress-strain curves plotted from observed data obtained in testing the used drill pipe in the condition as received and after heat treatment are shown in Figures 9 to 14, inclusive.

Although all of the samples have a tensile yield strength greater than the specification minimum of 75,000 p. s. i., samples H1, H2 and H5 show an appreciable Bauschinger effect in the compression tests. There is little difference between the compression and tensile curves of samples H4 and H6 in which the yield strengths are at a relatively high stress level. This shows that some of the used drill pipe samples were in worse condition than others.

TABLE 8  
Mechanical properties of drill pipe which had been  
used in drilling

| Specimen<br>Number | Temp.,<br>F. | Compression Yield Strength   |                             |                            | Tensile Yield Strength       |                             |                            | Ultimate<br>Tensile<br>Strength,<br>p. s. i. | Elonga-<br>tion,<br>percent |
|--------------------|--------------|------------------------------|-----------------------------|----------------------------|------------------------------|-----------------------------|----------------------------|----------------------------------------------|-----------------------------|
|                    |              | 0.02%<br>Offset,<br>p. s. i. | 0.2%<br>Offset,<br>p. s. i. | 0.5%<br>Total,<br>p. s. i. | 0.02%<br>Offset,<br>p. s. i. | 0.2%<br>Offset,<br>p. s. i. | 0.5%<br>Total,<br>p. s. i. |                                              |                             |
| H1                 |              | 30,000                       | 60,000                      | 65,000                     | 55,000                       | 81,000                      | 81,000                     | 109,000                                      | 20                          |
|                    |              | 30,000                       | 60,000                      | 64,000                     |                              |                             |                            |                                              |                             |
| H2                 |              | 40,000                       | 72,000                      | 75,000                     | 62,000                       | 91,000                      | 91,000                     | 117,500                                      | 18                          |
|                    |              | 42,000                       | 72,000                      | 75,000                     |                              |                             |                            |                                              |                             |
| H3                 |              | 65,000                       | 82,000                      | 82,000                     | 65,000                       | 78,000                      | 78,500                     | 110,000                                      | 21                          |
|                    |              | 65,000                       | 82,000                      | 82,000                     |                              |                             |                            |                                              |                             |
| H4                 |              | 55,000                       | 87,000                      | 87,000                     | 70,000                       | 87,000                      | 87,000                     | 116,500                                      | 20                          |
|                    |              | 55,000                       | 88,000                      | 89,000                     |                              |                             |                            |                                              |                             |
| H5                 |              | 40,000                       | 54,500                      | 60,000                     | 50,000                       | 80,000                      | 80,500                     | 109,500                                      | 23                          |
|                    |              | 40,000                       | 55,000                      | 61,000                     |                              |                             |                            |                                              |                             |
| H6                 |              | 89,000                       | 90,000                      | 90,000                     | 86,500                       | 87,500                      | 87,500                     | 118,000                                      | 19                          |
|                    |              | 90,000                       | 91,000                      | 91,000                     |                              |                             |                            |                                              |                             |

  

| AFTER HEATING FOR 1 HOUR AT 850 F. |     |        |        |        |         |         |         |         |    |  |
|------------------------------------|-----|--------|--------|--------|---------|---------|---------|---------|----|--|
| H1                                 | 850 | 83,000 | 83,000 | 83,000 | 91,000  | 91,000  | 91,000  | 110,500 |    |  |
| H2                                 | 850 | 92,000 | 92,000 | 92,000 | 101,000 | 101,000 | 101,000 | 119,000 | 23 |  |
| H3                                 | 850 | 87,000 | 88,500 | 88,500 | 85,500  | 85,500  | 85,500  | 113,500 | 20 |  |
| H4                                 | 850 | 90,000 | 90,000 | 90,000 |         |         |         |         |    |  |
| H5                                 | 850 | 81,000 | 81,000 | 81,000 | 91,000  | 91,000  | 91,000  | 112,000 | 24 |  |
| H6                                 | 850 | 93,500 | 93,500 | 93,500 | 91,000  | 91,000  | 91,000  | 118,500 | 20 |  |

The shape of the curve for tests showing low yield strengths is not typical of stress-free, low-strength material but has the long low sweep which has been demonstrated above to be characteristic of the steel when plastically pretrained in the direction opposite to the direction of testing. The beneficial effect of the heat treatment in restoring the properties of pipe damaged by plastic strains in field service is shown in the curves of Figures 9 to 14, inclusive.

A length of 3½ inch outside diameter 13.3-pound grade E seamless steel drill pipe was loaded as a cantilever beam and rotated 26,000 revolutions. Four compression and four tensile test bars were machined from the wall of the pipe at a location beyond the point of loading and thus represent the condition of the steel before fatigue-type loading. A similar set of specimens was machined from a location in the pipe stressed to 16,500 p. s. i. in the outer fibers and a third set from a location stressed to 31,000 p. s. i. in the outer fibers. The results of mechanical tests made on the bars are given in Table 9.

TABLE 9  
Mechanical properties of steel drill pipe after fatigue-type loading

| Specimen<br>Number | Yield Strength<br>0.2% Offset,<br>p. s. i. |         | Yield Strength<br>0.5% Total,<br>p. s. i. |         | Ultimate<br>Strength,<br>p. s. i. |  |
|--------------------|--------------------------------------------|---------|-------------------------------------------|---------|-----------------------------------|--|
|                    | Com-<br>pression                           | Tension | Com-<br>pression                          | Tension |                                   |  |
|                    |                                            |         |                                           |         |                                   |  |
| 1-A <sup>a</sup>   | 81,000                                     | 77,000  | 81,000                                    | 77,000  | 107,900                           |  |
| 1-B                | 81,000                                     | 74,150  | 81,500                                    | 74,250  | 103,100                           |  |
| 1-C                | 86,000                                     | 78,200  | 86,000                                    | 78,350  | 105,900                           |  |
| 1-D                | 89,500                                     | 75,700  | 89,500                                    | 76,000  | 105,900                           |  |
| 2-A <sup>b</sup>   | 85,000                                     | 73,000  | 87,000                                    | 74,000  | 107,200                           |  |
| 2-B                | 83,000                                     | 74,250  | 84,000                                    | 75,750  | 107,450                           |  |
| 2-C                | 82,000                                     | 71,500  | 82,500                                    | 73,750  | 108,000                           |  |
| 2-D                | 82,000                                     |         | 84,000                                    |         |                                   |  |
| 3-A <sup>c</sup>   | 83,000                                     | 72,000  | 84,500                                    | 73,000  | 105,050                           |  |
| 3-B                | 85,000                                     | 69,750  | 87,000                                    | 71,600  | 106,650                           |  |
| 3-C                | 79,000                                     | 69,250  | 80,500                                    | 70,900  | 105,450                           |  |
| 3-D                | 82,000                                     | 73,000  | 83,000                                    | 75,000  | 108,000                           |  |

<sup>a</sup> Specimens from a location in the pipe stressed to 31,500 p. s. i. in the outer fibers.

<sup>b</sup> Specimens from a location in the pipe stressed to 16,500 p. s. i. in the outer fibers.

<sup>c</sup> Specimens from a location in the pipe not stressed during the fatigue-type loading.

NOTE.—3½ inch O. D., 13.30#, Grade E seamless steel pipe loaded as a cantilever beam and rotated 26,000 revolutions.

30 Stress-strain curves typical of the tensile properties obtained from bars from the three locations mentioned are shown in Figure 15 and compression curves are shown in Figure 16. The relatively large radius of curvature at the nose of the curves for the material that had not been 35 fatigued indicates that some residual stress was present. If such residual stress was caused by prestraining, the prestraining was apparently not in a direction parallel to the longitudinal axis of the pipe because both the compression curve and the tension curve have the

40 same characteristics. The other curves of the figure show that if a sufficiently high stress is applied alternately in compression and in tension for the number of cycles mentioned the residual stresses will be relieved and the material will perform elastically to a much higher stress level. The results indicate that cyclic loading may be effective in removing the Bauschinger effect.

45 Experiments were conducted to determine the effect of repeated reverse strain beyond the elastic limits on the 50 mechanical properties of steel pipe. The specimens used were prepared from 3-inch long strips cut from the wall of a pipe in the normalized condition. The ends of the strips were built up by welding and turned and threaded to the standard ¾-inch thread used on the testing machine. The strip at the center of the bars was turned and ground on the same centers to the largest practicable diameter, approximately .35 inch. This formed a reduced section 1½ inches long at the center of the length 55 of the bars. Before each loading in compression the gauge length of the bars was held in a V-block and the two ends were reground parallel to each other and perpendicular to the axis of the bar.

60 Two of the bars were subjected to a total strain of approximately .5% and the load was released and applied in the opposite direction to the same total strain. The bars were cycled in this manner several times. However, one bar was started with a compression load and the other with a tension load. The second pair of bars was treated in the same manner except that such bars were strained to approximately 1% total elongation. The results of these tests are given in Table 10 and are 65 shown graphically in Figures 17 to 20, inclusive.

TABLE 10

Mechanical properties of steel strained alternately in opposite directions

0.320-INCH-DIAMETER BAR STRAINED APPROXIMATELY 0.5 PERCENT

|                  | 0.02%<br>Offset,<br>p. s. i. | 0.2%<br>Offset,<br>p. s. i. | 0.5%<br>Total,<br>p. s. i. |
|------------------|------------------------------|-----------------------------|----------------------------|
| Tension.....     | 77,500                       | 77,500                      | 77,500                     |
| Compression..... | 43,000                       | 71,000                      | 76,000                     |
| Tension.....     | 27,000                       | 66,000                      | 71,000                     |
| Compression..... | 83,000                       | 83,000                      | 83,000                     |

0.358-INCH-DIAMETER BAR STRAINED APPROXIMATELY 1.0 PERCENT

|                  | 0.02%<br>Offset,<br>p. s. i. | 0.2%<br>Offset,<br>p. s. i. | 0.5%<br>Total,<br>p. s. i. |
|------------------|------------------------------|-----------------------------|----------------------------|
| Tension.....     | 79,000                       | 79,000                      | 79,000                     |
| Compression..... | 29,000                       | 46,000                      | 53,000                     |
| Tension.....     | 20,000                       | 58,000                      | 65,000                     |
| Compression..... | 40,000                       | 69,000                      | 77,000                     |

0.348-INCH-DIAMETER BAR STRAINED APPROXIMATELY 0.5 PERCENT

|                  | 0.02%<br>Offset,<br>p. s. i. | 0.2%<br>Offset,<br>p. s. i. | 0.5%<br>Total,<br>p. s. i. |
|------------------|------------------------------|-----------------------------|----------------------------|
| Compression..... | 83,000                       | 83,000                      | 83,000                     |
| Tension.....     | 18,000                       | 52,000                      | 59,000                     |
| Compression..... | 35,000                       | 65,000                      | 70,000                     |
| Tension.....     | 25,000                       | 63,000                      | 68,000                     |
| Compression..... | 35,000                       | 62,000                      | 67,000                     |
| Tension.....     | 20,000                       | 57,000                      | 63,000                     |

0.340-INCH-DIAMETER BAR STRAINED APPROXIMATELY 1.0 PERCENT

|                  | 0.02%<br>Offset,<br>p. s. i. | 0.2%<br>Offset,<br>p. s. i. | 0.5%<br>Total,<br>p. s. i. |
|------------------|------------------------------|-----------------------------|----------------------------|
| Compression..... | 82,000                       | 82,000                      | 82,000                     |
| Tension.....     | 19,000                       | 64,000                      | 62,000                     |
| Compression..... | 42,000                       | 71,000                      | 75,000                     |
| Tension.....     | 27,000                       | 60,000                      | 67,000                     |

While I have described certain present preferred methods of practicing the invention it is to be distinctly understood that the invention is not limited thereto but may be otherwise variously practiced within the scope of the following claims.

I claim:

1. A method of restoring the elastic limit and yield strength of oil well drill pipe which has been reduced due to Bauschinger effect caused by cold plastic deformation in drilling operations which comprises heat treating said pipe within the temperature range of from 400° F. to 1250° F.

10 2. A method of restoring the elastic limit and yield strength of oil well drill pipe which has been reduced due to Bauschinger effect caused by cold plastic deformation in drilling operations which comprises heat treating the pipe at about 850° F. for about an hour.

15 3. A method of restoring the elastic limit and yield strength of oil well drill pipe which has been reduced due to Bauschinger effect caused by cold plastic deformation in drilling operations which comprises applying thereto energy relieving the microstresses within the atomic lattice.

25 References Cited in the file of this patent

UNITED STATES PATENTS

2,320,040 Landis May 25, 1943

30 OTHER REFERENCES

Zeitschrift für Metallkunde, vol. 17, 1925, pages 268-269. G. Masing.

Polakowski: Iron Age, August 28, 1952, pages 107-111.

UNITED STATES PATENT OFFICE  
CERTIFICATE OF CORRECTION

July 15, 1958

Patent No. 2,843,512

Joseph W. Lodge

It is hereby certified that error appears in the printed specification of the above numbered patent requiring correction and that the said Letters Patent should read as corrected below.

Column 2, line 18, for "grade E seamless drill pipe" read -- Grade E seamless drill pipe --; column 3, line 11, after "moderate" insert -- amount of residual internal stress show that the elastic --; line 14, strike out "amount of residual internal stress show that the elastic"; line 25, for "grade E" read -- Grade E --; column 4, line 35, for "prestraining" read -- restraining --; column 11, line 30, for "ypical" read -- typical --.

Signed and sealed this 11th day of November 1958.

(SEAL)

Attest:

KARL H. AXLINE  
Attesting Officer

ROBERT C. WATSON  
Commissioner of Patents